

Dec. 7, 1943.

T. G. McDUGAL ET AL

2,336,182

CERAMIC ARTICLE AND METHOD OF MAKING SAME

Filed May 31, 1940



McDUGAL  
Inventors

Teine G. McDugal &  
Karl Schwitzerwalt

By

Blackmores, Spence & Hink  
Attorneys

## UNITED STATES PATENT OFFICE

2,336,182

CERAMIC ARTICLE AND METHOD OF  
MAKING SAME

Taine G. McDougal and Karl Schwartzwalder,  
Flint, Mich., assignors to General Motors Cor-  
poration, Detroit, Mich., a corporation of Dela-  
ware

Application May 31, 1940, Serial No. 338,094

12 Claims. (Cl. 106—62)

This invention relates to ceramic bodies having compositions which lie in the ceramic oxide system  $\text{BeO}-\text{MgO}-\text{Al}_2\text{O}_3$  and to methods of making articles of such compositions. The preferred compositions are particularly adapted for use as insulators for spark plugs and the like which require one or more of the physical characteristics of high thermal conductivity, high thermal capacity, high thermal expansion, high dielectric strength at elevated temperatures and the ability to withstand sudden temperature changes. All of these physical characteristics are prerequisites of satisfactory spark plug insulators for automotive and aircraft engines.

Spark plug insulator bodies made according to this invention possess the indicated qualities to a high degree and in addition possess the great advantage that they may be fired at relatively low temperatures. This is important in commercial production as the equipment required to fire at high temperatures is both difficult and expensive to construct and maintain. The improved bodies are especially characterized by high thermal conductivity and high thermal expansion.

We have discovered that certain combinations of oxides in the triaxial systems

$\text{BeO}-\text{MgO}-\text{Al}_2\text{O}_3$

and the four component system

$\text{BeO}-\text{MgO}-\text{Al}_2\text{O}_3-\text{SiO}_2$

produce very excellent insulators at temperatures only slightly higher than those required for firing present-day commercial porcelains. The preferred combinations of oxides are disclosed in the triaxial diagram illustrated on the accompanying drawing.

Referring to the figure the area

A—B—C—D—E

contains the preferred spark plug insulator compositions in this system. This area corresponds to the following percentage range:

|                         | Per cent |
|-------------------------|----------|
| $\text{BeO}$            | 45-98    |
| $\text{MgO}$            | 1-25     |
| $\text{Al}_2\text{O}_3$ | 1-35     |

Bodies lying within this area have the most desirable combination of the above-mentioned physical properties in combination with relatively low firing temperatures. Thus, for example, point 1 on the diagram indicates a composition of 95%  $\text{BeO}$ , 2.5%  $\text{MgO}$ , 2.5%  $\text{Al}_2\text{O}_3$  having a firing temperature of Orton cone 30 (1650° C.) in

contrast with 2000° C. required for  $\text{BeO}$ . Increasing the percentage of  $\text{MgO}$  and  $\text{Al}_2\text{O}_3$  lowers the sintering temperature. Thus, point 2 on the diagram indicates a composition of 90%  $\text{BeO}$ , 5%  $\text{MgO}$ , 5%  $\text{Al}_2\text{O}_3$  having a sintering temperature of Orton cone 23 (1580° C.). Point 3 indicates a composition of 60%  $\text{BeO}$ , 20%  $\text{MgO}$ , 20%  $\text{Al}_2\text{O}_3$  having a sintering temperature of Orton cone 20 (1530° C.) which is only slightly higher than that required for conventional porcelain spark plug insulators.

Spark plug insulators made from these new compositions have such greater thermal conductivity and thermal capacity that, in measurements in terms of insulation length required for spark plug insulators, they are six to seven insulation lengths better than the best grade of spark plug porcelain. That is, an insulator of the new composition 6 or 7/32 of an inch longer than the best porcelain insulator will perform as well as such porcelain insulator with respect to the said thermal qualities. They are also superior in this respect to any of the increasingly used sintered oxide insulators with which we are familiar. At the same time no breakage occurs due to thermal shock and the electrical resistance at high temperatures is considerably higher than that of porcelains now in general use. The thermal expansion is also greater, an advantage in that it more nearly approximates that of the metal housing in which the insulator is assembled to form the complete compression-tight spark plug. It is indicated that these new compositions may provide as great improvement for such uses as radio work where low power factor loss is necessary as they do for spark plug insulators.

The next best bodies have compositions lying within the area F—G—H—I on the diagram. This area corresponds to the following composition range:

|                         | Per cent |
|-------------------------|----------|
| $\text{BeO}$            | 15-40    |
| $\text{MgO}$            | 15-40    |
| $\text{Al}_2\text{O}_3$ | 45-65    |

As an example, the composition indicated at point 4, 20%  $\text{BeO}$ , 30%  $\text{MgO}$ , 50%  $\text{Al}_2\text{O}_3$ —fires to a non-porous structure at Orton cone 20 (1530° C.). The physical characteristics of these bodies are very similar to those of the compositions previously mentioned, being greatly superior to those of present-day commercial porcelain insulators.

A third area which gives compositions having good physical characteristics but considerably lower than the two areas previously described is

designated by area J—K—L, corresponding to the following range of percentages:

|                                | Per cent |
|--------------------------------|----------|
| BeO                            | 1-10     |
| MgO                            | 1-10     |
| Al <sub>2</sub> O <sub>3</sub> | 88-98    |

The bodies within the three areas above specified are especially adapted for use as spark plug insulators. For many other uses such as crucibles, and insulators other than for spark plugs, the same physical characteristics are not required. Very useful bodies for such purposes will be found throughout the area designated A—L—X—W corresponding to the following percentage range:

|                                | Per cent |
|--------------------------------|----------|
| BeO                            | 1-98     |
| MgO                            | 1-40     |
| Al <sub>2</sub> O <sub>3</sub> | 1-98     |

The bodies within this larger area all possess high thermal conductivity, high temperature electrical resistance, and excellent thermal shock resistance.

A further embodiment of the invention consists in the addition of SiO<sub>2</sub> to the bodies just described. This results in a further lowering of the firing temperature without detracting greatly from the desirable physical characteristics of the product and in some cases improving them. In general we have found it preferable to maintain the silica content below 20% although good insulators have been made with somewhat higher silica contents.

The following are examples of the quaternary bodies just discussed. A body consisting of 5% BeO, 20% MgO, 60% Al<sub>2</sub>O<sub>3</sub>, 15% SiO<sub>2</sub> matures at Orton cone 20 (1530° C.), as compared with 1785° C. for the same body with the silica omitted. At the same time the resistance of the body to thermal shock breakage is greatly improved.

The addition of 7.6% silica to a body consisting of 39% BeO, 4% MgO, 57% Al<sub>2</sub>O<sub>3</sub> reduces the sintering temperature from Orton cone 35 (1785° C.) to Orton cone 20 (1530° C.) while maintaining the desirable physical characteristics.

The materials required for the bodies may be added as oxides or as various compounds or compositions having different mineralogical forms, such as silicates, spinel, aluminates and so on and it will be understood that where in the claims the bodies are defined by oxide content such variations are contemplated as equivalents. It will also be understood that small proportions of suitable known ceramic fluxes or diluent materials may be added when desired in accordance with well-known practices in the ceramic art. The following are some examples of the forms in which the raw materials may be introduced into the batch:

#### Beryllia.

Beryllia, preferably low in alkalies, may be added as the chemically precipitated beryllium oxide, raw or calcined; or as synthetic beryllium aluminate; or, when silica is to be present, as beryl or other beryllium containing minerals, or as a by-product from the treatment of beryllium minerals to obtain the metals.

#### Magnesia

Magnesia is preferably added in a pure form such as electric furnace periclase; as magnesite or prepared magnesium carbonate; as natural or prepared hydrated magnesia, preferably cal-

cined to form periclase; as prepared magnesium aluminate. When silica is to be present the magnesia can be added as magnesium silicates such as talc or magnesium aluminum silicates.

#### Alumina

Alumina is preferably added as calcined alumina prepared by the Bauer process; as calcined diaspor or bauxite; as electric furnace or high temperature calcined alumina. When silica is to be present, clay, minerals of the sillimanite group, or other aluminum silicates, synthetic aluminum silicates, or alkali earth aluminum silicates, may be added.

#### Silica

Silica is preferably added as amorphous silica, quartz, cristobalite, or tridymite; in a combined form, natural or synthetic, such as beryllium, or magnesia or aluminum silicates or as beryllium magnesium silicate.

Articles produced from the compositions specified may be processed in the manner described in U. S. Patent 2,091,973, issued to Fessler and Russell on September 7, 1937, or in our Patent

No. 2,122,960, granted to Schwartzwalder on July 5, 1938; or by casting in molds; or by extrusion and grinding the dried extruded blank; or in compositions in which clay is used to introduce Al<sub>2</sub>O<sub>3</sub> and SiO<sub>2</sub>, by other methods well known to ceramic art, such as dry-pressing, pugging and grinding or turning. The usual organic plasticizers or inorganic gels or zeolites may be added to aid fabrication.

The raw materials employed in the body compositions should be in a very fine state of subdivision, preferably all the material finer than 43 microns with a greater portion lying between 0 and 5 microns.

In our preferred method of forming, disclosed in said Schwartzwalder patent, the inorganic materials are ground with a suitable proportion of temporary organic binder, such as Bakelite, together with a lubricant. The finely ground material is then granulated and preformed into predetermined shapes. These shapes are then assembled on a center pin placed in the die and pressed into insulator shapes under heat and heavy pressure. Setting of the binder produces a firm shape readily handled in mass production facilitating the subsequent manufacturing operations. The formed body is fired to a sufficiently high temperature to eliminate the organic binder and to recrystallize the mass into a fine-grained dense impervious structure.

We claim:

1. A ceramic product made by firing a ceramic mixture showing upon chemical analysis approximately from 1 to 98% beryllium oxide, from 1 to 40% magnesium oxide and the balance alumina together with up to 20% silica.

2. An insulator for spark plugs and the like characterized by high thermal conductivity, high thermal capacity, high thermal expansion, high dielectric strength at elevated temperatures, high thermal shock resistance and good mechanical strength made by firing to a dense, non-porous state, an insulator shape formed from a batch consisting of a finely pulverized mixture showing upon chemical analysis approximately from 45 to 98% beryllium oxide, from 1 to 25% magnesium oxide and from 1 to 35% aluminum oxide.

3. An insulator for spark plugs and the like characterized by high thermal conductivity, high

thermal capacity, high thermal expansion, high dielectric strength at elevated temperatures, high thermal shock resistance and good mechanical strength made by firing to a dense, non-porous state, an insulator shape formed from a batch consisting of a finely pulverized mixture showing upon chemical analysis approximately from 45 to 98% beryllium oxide, from 1 to 25% magnesium oxide, from 1 to 35% aluminum oxide and up to 20% silica.

4. An insulator for spark plugs and the like characterized by high thermal conductivity, high thermal capacity, high thermal expansion, high dielectric strength at elevated temperatures, high thermal shock resistance and good mechanical strength made by firing to a dense, non-porous state, an insulator shape formed from a batch consisting of a finely pulverized mixture showing upon chemical analysis approximately from 15 to 40% beryllium oxide, 15 to 40% magnesium oxide and from 45 to 65% aluminum oxide.

5. An insulator for spark plugs and the like characterized by high thermal conductivity, high thermal capacity, high thermal expansion, high dielectric strength at elevated temperatures, high thermal shock resistance and good mechanical strength made by firing to a dense, non-porous state, an insulator shape formed from a batch consisting of a finely pulverized mixture showing upon chemical analysis approximately from 15 to 40% beryllium oxide, 15 to 40% magnesium oxide, from 45 to 65% aluminum oxide and up to 20% silica.

6. An insulator for spark plugs and the like characterized by high thermal conductivity, high thermal capacity, high thermal expansion, high dielectric strength at elevated temperatures and high thermal shock resistance and good mechanical strength made by firing to a dense, non-porous state, an insulator shape formed from a batch consisting of a finely pulverized mixture showing upon chemical analysis approximately from 1 to 10% beryllium oxide, from 1 to 10% magnesium oxide, from 88 to 98% aluminum oxide and up to 20% silica.

7. A ceramic product made by firing a ceramic mixture showing upon chemical analysis approximately from 1 to 98% beryllium oxide, from 1 to 40% magnesium oxide and the balance alumina together with 0 to 20% silica.

8. Ceramic product made by firing to dense, non-porous state a compacted body formed of a ceramic mixture showing upon chemical analysis approximately from 1 to 98% beryllium oxide, from 1 to 40% magnesium oxide and the balance alumina.

9. Ceramic product made by firing to dense, non-porous state a compacted body formed of a ceramic mixture showing upon chemical analysis approximately from 1 to 98% beryllium oxide, from 1 to 40% magnesium oxide, up to 20% silica and the balance alumina.

10. An insulator for spark plugs and the like made by firing to a dense, non-porous state a compacted insulator shape formed from a finely pulverized ceramic mixture showing upon chemical analysis approximately from 1 to 98% beryllium oxide, from 1 to 40% magnesium oxide, and the balance alumina.

11. The method of making spark plug insulators and the like which consists in preparing a finely pulverized ceramic mixture showing upon chemical analysis approximately from 1 to 98% beryllium oxide, from 1 to 40% magnesium oxide and the balance aluminum oxide, forming the mixture into the shape of the desired article, and thereafter firing the shape to sinter it into a dense, non-porous insulator body.

12. The method of making spark plug insulators and the like which consists in preparing a finely pulverized ceramic mixture showing upon chemical analysis approximately from 1 to 98% beryllium oxide, from 1 to 40% magnesium oxide, from 0 to 20% silica, and the balance aluminum oxide, forming the mixture into the shape of the desired article, and thereafter firing the shape to sinter it into a dense, non-porous insulator body.

TAINIE G. McDUGAL,  
KARL SCHWARTZWALDER.